

# UNITED STATES PATENT OFFICE.

JAMES E. GILLESPIE, OF WARWICK, NEW YORK.

## WATERPROOFING AND PRESERVATIVE COMPOUND.

SPECIFICATION forming part of Letters Patent No. 253,369, dated February 7, 1882.

Application filed December 8, 1881. (No specimens.)

*To all whom it may concern:*

Be it known that I, JAMES E. GILLESPIE, of Warwick, in the county of Orange and State of New York, have invented a certain new and 5 Improved Waterproofing and Preservative Compound, of which the following is a specification.

My improved compound is applicable to fabrics made of fibrous material by felting, weaving, or otherwise, to leather and to wood, or other materials.

The invention consists in a waterproofing and preservative compound composed of ozocerite or mineral wax and a siccative vegetable oil—such, for instance, as linseed-oil. The proportions which I have used successfully are one (1) part, by weight, of ozocerite or mineral wax, and two (2) parts, by weight, of linseed-oil, cotton-seed oil, or any other suitable siccative 15 vegetable oil. These proportions may, however, be varied for treating different substances under varying conditions.

The compound is made by placing the ozocerite and oil together in a suitable vessel heated 25 to a temperature sufficient to melt the ozocerite and enable it to be incorporated with the oil, which is about one hundred and eighty degrees (180°) Fahrenheit, or upward.

The fabric or other material to be waterproofed and preserved is treated in the following manner: The compound of ozocerite and oil heated sufficiently to render it fluid is ap-

plied to the surface of the fabric or material with a brush or by any other means, and the fabric or material is then placed in a chamber 35 or other place heated to a temperature of from one hundred and fifty degrees (150°) to two hundred and fifty degrees (250°) Fahrenheit, and allowed to remain therein for a very short time to allow the ozocerite and oil to strike into 40 and thoroughly penetrate the fabric or material. This application of ozocerite and oil and the subsequent heating may be repeated when necessary, and as often as is desirable.

The ozocerite and oil may be applied with 45 great advantage to seamless woven hose.

I do not here claim the use of ozocerite alone as a waterproofing substance, as this may form the substance of a future application for Letters Patent.

What I claim as my invention, and desire to 50 secure by Letters Patent, is—

1. A waterproofing and preservative compound composed of ozocerite or mineral wax and a siccative vegetable oil, substantially as 55 herein described.

2. A waterproofing and preservative compound composed of ozocerite or mineral wax and linseed-oil, substantially as herein described.

JAMES E. GILLESPIE.

Witnesses:

FREDK. HAYNES,  
EDWARD GLATZMAYER.